

Feb. 10, 1970

KATSUO MAKINO ET AL

3,494,789

PHOTOCONDUCTIVE INSULATING MATERIAL

Filed June 2, 1966

3 Sheets-Sheet 1

FIG. 1



SURFACE POTENTIAL

INVENTORS  
KATSUO MAKINO  
IWAO SAWATO

BY

*Sugrus, Rothwell, neon, Zeni, & Macpeak*

ATTORNEYS.

Feb. 10, 1970

KATSUO MAKINO ET AL

3,494,789

PHOTOCONDUCTIVE INSULATING MATERIAL

Filed June 2, 1966

3 Sheets-Sheet 2

FIG. 2



*Suguru Rockwell, Nixon, Zinn & Macpeak*  
ATTORNEYS.

Feb. 10, 1970

KATSUO MAKINO ET AL

3,494,789

PHOTOCONDUCTIVE INSULATING MATERIAL

Filed June 2, 1966

3 Sheets-Sheet 3

FIG. 4



INVENTORS.  
KATSUO MAKINO  
IWAO SAWATO

BY

Sugihara, Rothwell, Nixon, Finn & Nease, Inc.  
ATTORNEYS.

# United States Patent Office

3,494,789

Patented Feb. 10, 1970

1

3,494,789

PHOTOCONDUCTIVE INSULATING MATERIAL  
Katsuo Makino and Iwao Sawa, Kanagawa, Japan, assignors to Fuji Shashin Film Kabushiki Kaisha, Kanagawa, Japan

Filed June 2, 1966, Ser. No. 554,840

Claims priority, application Japan, June 2, 1965,  
40/32,170

Int. Cl. B44d 1/18, 1/34

U.S. Cl. 117—201

2 Claims

## ABSTRACT OF THE DISCLOSURE

The invention is directed to a photoconductive insulating material mainly used for electrophotography. Said material comprises an electrically insulating binder material having a bulk resistivity of at least  $10^{11}$  ohm-cm. at room temperature, and dispersed therein finely divided particles of the reaction product of cadmium carbonate and sulfur.

This invention relates to a photoconductive insulating material mainly used for electrophotography.

As the photoconductive insulating material used for electrophotography, it has been known to employ some sort of photoconductive inorganic compounds.

Such substances, for example, as sulfur, selenium, and further compounds, such as oxides, sulfides, or selenides of zinc, cadmium, mercury, bismuth, lead, etc., and also titanium oxide are known. Those substances are coated stratiformly on a plate, e.g., a metal plate, paper and so on. If necessary, the photoconductive insulating layer could be formed by dispersing these substances in the electric insulating resin binder. Among these substances, selenium and zinc oxide are the best known and are practically used up to now.

The procedure to get an electrophotographic image on the electrophotographic sensitive body having a photoconductive insulating layer employing these substances first begins with the placing of an electrostatic charge on the surface of the photoconductive insulating layer to bestow photosensitivity by corona discharge for instance, in the dark. Next follows exposure by usual photographic procedure. The latent image got by exposure is then developed with charged toning powder into the visible image. The toning powder image is fixed intact upon the layer of photoconductive insulating material or alternatively transferred upon other suitable supporting body and fixed. When the image is transferred, the residual toning powder on the layer of the photoconductive insulating material is swept away so that the said layer could be reused. The above-mentioned process is a most general one in the art of electrography and further, pluralities of modified process or many kinds of methods and means to enable those processes are being considered, but fundamental properties of those photoconductive insulating layers could be regarded essentially as identical.

Selenium, now widely known and employed for practical use, is employed as a reusable photosensitive material coated on a metal plate, particularly on an aluminum plate, in the form of vitreous selenium layer. The photosensitivity of it corresponds to ASA 2-10 which is considered to be the highest among those electrophotographic sensitive materials up to now. In addition, the vitreous selenium is exceedingly well fitted for practical reuse because it has a very hard, mirror surface. On the other hand, another practically utilized zinc oxide is used to form an electrographic sensitive body, called a photosensitive paper, by a process of dispersing it in an electric insulating resin binder and coating it on a sheet of paper

2

which is then dried. This photosensitive paper, having a photosensitivity in the range of about ASA 0.01-0.2, looks almost white so that an image could be formed and fixed directly upon the paper. The said dispersed layer of zinc oxide could be also coated on a metal body, but it has not been used as a reusable photosensitive material for the reasons that it is far inferior to a photosensitive material employing selenium in such properties as lower film hardness and lower photosensitivity.

Moreover, once exposed to light, the properties of the layer are impaired to a state unfit for continuous and repeated use. Other than selenium and zinc oxide, only the properties of titanium oxide in practical use have been reported.

We should designate one method, the direct image producing process, comprising fixing the toning powder directly on the layer of photoconductive insulating material. Another method may be designated the indirect image producing process. This comprises either fixing the transferred image on other transferring material which is formed on the layer of photoconductive insulating material or developing and fixing on the transferred material, after transferring of the latent electrostatic image, formed on the layer of the photoconductive insulating material, to other transferring material, i.e., the method to form an image on other material with an aid of the layer of photoconductive insulating material.

In the direct image producing process, though it has some advantages resulting from its own properties, the layer of photoconductive insulating material imposes limitations in regard to the whiteness which is possible in copying the documents and the pliability of the coated sheet, for example, a paper. The whiteness of photoconductive insulating layer does not cause any problem in getting a copy image consisting of black and white, but it becomes a fatal defect in copying color printed matter. It could be understood that the limitation of employing a supporting body of paper and the like prevents the material from fully exhibiting the special properties of a photoconductive insulating layer. On the contrary, in the indirect image producing process, there is almost no limitation in employing the color and kinds of the supporting body of the photoconductive insulating layer, and they may be freely chosen so that there becomes possible combinations by which each special characteristic could be exhibited fully. And further, in the latter process an additional advantage exists, i.e., the possibility of continuous and repeated use.

It has previously been known to employ vitreous selenium as an electrophotographic sensitive material for continuous and repeated use. The said material has excellent properties such as photosensitivity, film hardness and pre-exposure effect, as the photoconductive insulating layer. On the other hand, some defects, for example, the extreme difficulty in producing it, exist. Nowadays, it is formed by depositing on a plate by vacuum deposition as a film of uniform vitreous selenium, and the necessity of a large sized vacuum evaporating apparatus for manufacturing it has become the cause of lowering production efficiency. As an additional defect, controlling additive elements added for improving the properties, such as photosensitivity, becomes extremely difficult by vacuum evaporating process. Moreover, the vitreous selenium, being a sort of solid phase of selenium in a super-cooled state, tends to crystallize by heat, the moisture in air or contamination with other substances, which bring undesirable results to its properties with accelerated impairment of qualities and shortened life when used in high temperature and high humidity. However, in the case of employing zinc oxide, some trials for promoting photosensitivity by adding certain dyes have been done, but those dyes are thermally weak, and the deterioration of

properties by corona discharge and light radiation in continuous and repeated use is relatively rapid.

Therefore, the material still is inferior to selenium sensitive material at the point of short life for useful time.

To overcome the above-mentioned disadvantages, a layer of photoconductive insulating material has been developed and prepared by dispersing a photoconductive powder of cadmium sulfide whose mean particle size is about  $0.2\mu$ , in a solvent solution of a thermosetting resin having volume specific resistivity at least more than  $10^9$  ohm-cm., and coating it on a suitable plate, i.e., a metal plate, and promoting the hardening by baking while the heat treatment of the powder of cadmium sulfide and the resin system is done simultaneously. The photoconductive cadmium sulfide employed in this desirably does not contain any impurity and is a stoichiometrically perfect compound.

But so far as using such a kind of cadmium sulfide powder, it has been found that using it for a short period continuously and repeatedly is unsatisfactory because of the disadvantage of a too late response speed of photocurrent.

An object of this invention is to overcome these disadvantages inherent in vitreous selenium, zinc oxide and cadmium sulfide, etc., and further lies in proposing an improved photoconductive insulating material which has a photosensitivity equal to or more than that of vitreous selenium, and which is thermally stable, having a sufficiently low pre-exposure effect, being endurable in repeated and continuous use, as well as proposing a simple method of producing the said material.

In the accompanying drawing:

FIG. 1 shows the decay of the electrostatic potential of the surface of the electrophotographic sensitive materials of an example according to this invention and the prior art known hitherto;

FIG. 2 shows the relation between the initial surface potential and the exposure time for half decay, of the electrophotographic materials prepared according to one example of the invention and made of pure cadmium sulfide;

FIG. 3 illustrates the comparison of the variation of the surface potential immediately after charging (I.P.) in the case of employing continuously and repeatedly with the period of 10 sec. for one cycle, and that of the surface potential after exposure (R.P.) in repeated and continuous use, each for the photosensitive materials made of pure cadmium sulfide and of the example according to the invention; and

FIG. 4 shows the diagrammatic record of the X-ray diffraction analysis for the photoconductive powder used in an example of the invention, compared with that of pure cadmium sulfide.

Usually, an electrophotographic photosensitive body, which is prepared by coating a photoconductive insulating material onto a supporting member, is charged in one polarity by a corona discharger and it is not used in another polarity. The charging polarity is decided by the potential acceptance and the light sensitivity of the photosensitive member. Vitreous selenium, for example, is charged with positive ions and zinc oxide and cadmium sulfide with negative ions. But, by adding tellurium to vitreous selenium, some new electrophotographic sensitive material is considered whose photosensitivity is almost equal when charged either positive and negative and whose charge ability is almost equal in positive and negative charge by inserting an inter-layer between the supporting body and photo-conductive insulating layer. In the case that either positive and negative polarity is usable, an advantage lies in being able to get the directly developed image (negative  $\rightarrow$  negative or positive  $\rightarrow$  positive) and the reversibly developed image (negative  $\rightarrow$  positive or positive  $\rightarrow$  negative) by only changing the polarity of the corona discharge. A further object of this invention exists

in offering a photoconductive insulated material fitted for the use in either the positive and the negative charge.

Hereafter, a description is made mainly of what is fitted for use in electrophotography, but there will be wide usage beside it such as for example, in converting means of light or radiation signals into electrical signals as in a photocell, photoamplifier, image converter, phototape, etc., and also where powdered photoconductive insulating materials are dispersed in a suitable binder.

For instance, in electrophotography, to which this invention is applied, a description is made in the case of employing a Xerox Processor Model 914.

In the machine, a cylindrical electrographic sensitive body, which is coated with photoconductive insulating substance on its surface, is forced to rotate at constant speed in continuously and repeated use. It completes one cycle of the process by steps consisting of (1) charging, (2) exposing, (3) developing, (4) transferring, (5) cleaning off, (6) pre-exposing. The step of (6) pre-exposing, 10 is for the sake of accomplishing the preparation for proceeding the operation into the next cycle by discharging all the residual surface charges. The photosensitive body rotates a round in about 11 seconds. That is, within the period of 11 seconds, the process is performed repeatedly. It takes 10.4 secs. from after the step of (2) exposing 15 to the step of (1) charging of next cycle, during this time there is required the complete dissipation of the influence caused by the step (2) exposing. Further, the pre-exposure step (6) of the previous cycle should be performed before the charging step (1) and the allowed time 20 for it is only 0.6 sec. Therefore, the electrophotographic sensitive material must at least be able to reach the state in 0.6 sec. where nothing of the influence of the exposing effect is left. The photosensitive material prepared by 25 dispersing the powder of pure cadmium sulfide in a thermosetting resin and coating it on a metal plate which then is hardened by a heat treatment, could not be employed satisfactorily in Xerox Processor Model 914. However, electric charge ability in the dark and the photo-sensitivity is sufficiently high.

This is attributed to the response speed of photoelectric current. Particularly, the decaying time constant of photocurrent is approximately 2 sec., by half value time, so that though the dark resistance has remained in a lower state at 30 the time of charging (1), after pre-exposure (6) of the previous cycle, and the chargeability is lowered, the surface charge of the place that corresponds to the shadow part of the exposure decreases rapidly during a period of 3-4 sec. until the end of developing process, after charging 35 process. Thus, electrostatic contrast is lowered respectively and consequently. A disadvantage is the lowering of the contrast of the copied image.

To explain this phenomena, FIG. 3 should be employed where the abscissa represents the number of continuous repetitions in the case of using in the course of the aforementioned process with the period of 10 sec., and the ordinate represents the degree of surface potential immediately after the charging (1) designated I.P., and that at the time point corresponding to the end of the developing process, designated R.P. From the diagram, it should be understood that in the case of employing the photosensitive material #A-13 which is made of pure cadmium sulfide, the said I.P. decreases rapidly after only a few times of use.

We inventors have found the fact that instead of powder of cadmium sulfide a material comprising cadmium sulfide incorporated with cadmium carbonate has a relatively rapid response time to photocurrent and an electro-photosensitive member produced by dispersing it in an insulating resin and coating on a metal supporting body 45 has sufficient potential acceptance in the dark as well as high photosensitivity. Moreover, such photosensitive material could be charged either in positive or in negative polarity, as well as having sufficient photosensitivity. The 50 powder consisting of cadmium sulfide and cadmium car-

bonate can be produced by firing cadmium carbonate with sulfur powder at the temperature range between 400-600° C. As practical methods for this process, there is a pot firing or a calcination of cadmium carbonate in sulfur vapor. By employing a wet method, it would be obtained as a precipitant by dropping an aqueous solution of cadmium chloride into an aqueous solution of ammonium carbonate and ammonium sulfide.

## EXAMPLE 1

A fine powder consisting of cadmium sulfide and cadmium carbonate was obtained by firing the mixture of 0.1~0.2 micron diameter cadmium carbonate powder (70 weight parts) and sulfur fine powder (30 weight parts) at the temperature about 450 C. Some results of X-ray diffraction analysis of the photoconductive powder, thus obtained, is shown in FIG. 4. Accordingly, it could be understood that there exists a considerable amount of cadmium carbonate as well as cadmium sulfide as a polymorphous mixture of its hexagonal, cubic and amorphous, and the constitutional ratio of cadmium sulfide and cadmium carbonate ( $CdS \cdot XCdCo_3$ ) is approximately  $X \sim 1.5$ . Then, 155 g. of said powder is dispersed in 138.5 g. of thermoplastic acrylic resin solution commercially named Magicron #200 clear (48.9% of which is solid), which is available from Kansai Paint Company, with its thinner as a solvent. The material is mixed in a ball mill sufficiently to obtain a photosensitive paint. The paint is coated on an aluminum sheet which is dried preparatorily for 30 min. at 70° C. After drying, a further heat treatment for 30 min. at 150° C., is done and thus a photoconductive insulating layer having high film hardness is generated. As a typical example of an electrophotographic property inherent in electrophotographic sensitive member #1445, thus obtained, the variation of the surface potential is shown in FIG. 1. FIG. 1 also shows the decrease of surface potential of an electrophotographic member employing vitreous selenium, member #1001 comprising CdS and a binder, and the member #B2C comprising a dye-sensitized ZnO and a binder. Each ordinate of FIG. 1 is plotted logarithmically with a value of the surface potential for each sensitive member. The abscissa is plotted with a time by second unit, passed after charging.

Selenium is a most excellent material at the surface potential property in the dark and photosensitivity but, it is said so only when selenium is charged with positive and when charged negative, its property is very undesirable,

found that the potential acceptance increases in proportion to the film thickness, but the photosensitivity decreases as the film thickness increases.

Consequently, the initial surface potential, when charged in the dark, increases proportionately to the film thickness, and the amount of exposure to light required to reduce the potential to half of the initial state increases. A relation between the exposure time for half decaying of the potential and the initial surface potential in cases of varying them by changing the film thickness is such as shown in FIG. 2. For convenience of comparison, the data of photosensitive paint #D-60 which consists of pure cadmium sulfide, is also illustrated in FIG. 2. From FIG. 2, materials having satisfactory early surface potential and exposure time for half-decay could be determined for the purpose of obtaining a desired electrostatic contrast. The measurement conditions in FIG. 2 is as follows: (1) charging was done by corona-discharge at  $\pm 7.0$  kv. and, (2) exposure by tungsten lamp of 2666° K., where the intensity of illumination of a sample surface was above 15 lux. The aforementioned photosensitive pigment D-52 was coated on the outer surface of an aluminum pipe having a diameter about 200 mm. by a spray method, which was then dried for 30 min. at 70° C., after drying, it was heat-treated for 30 min. at 150° C. Thus, a cylindrical, reusable electrophotographic sensitive body was produced, whose coated film thickness was about 3.1 mg./cm.<sup>2</sup> after the heat-treatment. FIG. 3 shows the results from measuring the variation of the surface potential of said material in a method as described formerly, for example, in Xerox Processor Model 914, in the case of employing it continuously and repeatedly with a period of 10 sec. for one cycle. Charging is done by applying -6.5 kv. or -7.5 kv. to a single wire corotron and exposing to light was done at 250 lux sec., once. The initial surface potential immediately after the charging process (1) (I.P.) decreases rapidly early in several repeated uses in the case when photosensitive member #A-13 made of pure cadmium sulfide is used, but in the case of employing #A-25, according to an example of this invention, such variation can be scarcely observed in repeated use. The surface potential after exposure (R.P.) at the time point corresponding to the finished time of developing is shown only for #A-13, but for #A-25, it is too small to be illustrated and it hardly varies during repeated use. The values at the first time and the thirtieth time of repeated use are all as follows, as shown in Table 1.

TABLE 1

| Photosensitive member | Voltage of corona discharge, kv. | Initial surface potential (I.P.) |                  | After exposure surface potential (R.P.) |                  |
|-----------------------|----------------------------------|----------------------------------|------------------|-----------------------------------------|------------------|
|                       |                                  | 1st time, volts                  | 30th time, volts | 1st time, volts                         | 30th time, volts |
| #A-13-----{           | -6.5                             | 720                              | 400              | 25                                      | 10               |
| A-25-----{            | -7.5                             | 880                              | 575              | 36                                      | 22               |
|                       | -6.5                             | 680                              | 670              | 3                                       | 5                |
|                       | -7.5                             | 720                              | 710              | 4                                       | 4                |

though not shown in FIG. 1. CdS and ZnO exhibit excellent properties in negative charge. On the other hand, the photosensitive member #1445, an example of this invention, exhibits exerting properties either in positive and negative charge. The measurements in above cases were performed under the following conditions: (1) the applied potential for the charging by corona-discharge is 7.0 kv. either in positive or negative case, and (2) exposure was performed by a tungsten lamp at 2666° K. of its color temperature.

The intensity of the illumination on the surface of a sample was about 15 lux. In the course of examining the chargeability and photosensitivity of the sensitive pigment D-52, an example of this invention, coating it on an aluminum plate in various film thicknesses, it was

65 FIG. 3 and Table 1 show that in a photosensitive member of the example according to this invention, the response time of the photocurrent and, particularly, the decaying time constant of the photocurrent have been improved to be shorter than that of a photosensitive member employing CdS, and to a degree where no inconvenience exists in practical use with such a repeating period as is encountered in employing Xerox Processor Model 914.

70 There exists an optimum ratio for mixing the resin, as binder of the photosensitive layer and the photo-conductive powder, and the range of mixing ratio of practically usable materials are alike to the photoconductive insulating material comprising other photoconductive powders and resin binders.

## EXAMPLE 2

The same photoconductive powder comprising cadmium sulfide and cadmium carbonate,



as employed in Example 1 is used. As an insulating binder there is used a mixture of a silicone resin KR-211 (available from Shinetsu Chemical Industries Co. Ltd.), a room temperature drible resin binder, and an epoxyester (available from Nippon Oil and Fats Co. Ltd.). The photoconductive powder and the binder mixed at a ratio shown in Table 2, were mixed and kneaded in a porcelain ball-mill to disperse the powder, and thus photosensitive paints were produced. The said photosensitive paints were coated on an aluminum sheet of 0.1 mm. thickness by a spray-method, and were dried at room temperature. The amount of coated film after drying weighed 3.5-4.0 mg./cm.<sup>2</sup>.

TABLE 2.—PREPARATION CONDITIONS OF PHOTOSENSITIVE PAINTS

| Number of photo-sensitive paint | Photoconductive powder, g. | Silicone KR-211, g. | Epoxy-ester, J. | Toluol, cc. |
|---------------------------------|----------------------------|---------------------|-----------------|-------------|
| D-136                           | 98                         | 22.9                | 48              | 50          |
| D-160                           | 88                         | 22.9                | 48              | 50          |
| D-161                           | 78                         | 22.9                | 48              | 50          |
| D-162                           | 68                         | 22.9                | 48              | 50          |
| D-163                           | 58                         | 22.9                | 48              | 50          |

TABLE 3.—PROPERTIES OF ELECTROPHOTOGRAPHIC SENSITIVE MATERIALS PRODUCED EMPLOYING THE PHOTOSENSITIVE PIGMENT SHOWN IN FIGURE 2.

Charged -7.6 kv. by Corona Discharge  
Pre-exposure: 2000 Lux, 2 min. (Fluorescent Lamp)  
Measurement of Photosensitivity: Lux, Tungsten Lamp (2,660° K.)

| Number of photo-sensitive pigment | Rest     |            | At 15 sec. after pre-exposure |            | At 5 min. after pre-exposure |            | Exposure time for half decay, sec. |
|-----------------------------------|----------|------------|-------------------------------|------------|------------------------------|------------|------------------------------------|
|                                   | I.P., v. | D.D., min. | I.P., v.                      | D.D., min. | I.P., v.                     | D.D., min. |                                    |
| D-136                             | 320      | 0.62       | 330                           | 0.53       | 300                          | 0.63       | 2.77                               |
| D-160                             | 360      | 1.01       | 300                           | 0.80       | 370                          | 1.00       | 2.71                               |
| D-161                             | 360      | 1.20       | 380                           | 1.11       | 330                          | 1.10       | 3.66                               |
| D-162                             | 450      | 1.87       | 460                           | 1.85       | 440                          | 1.62       | 15.0                               |
| D-163                             | 530      | 2.10       | 570                           | 2.22       | 550                          | 2.25       | 30.0                               |

I.P.=Initial surface potential.  
D.D.=Dark half decay time.

Some measurement results of properties of the members, thus prepared, are shown in Table 3. Employing the said table, we should explain how the mix ratio of a resin, working as a binder of a photoconductive paint, and a photoconductive powder affects the characteristics of the product when employed as an electrophotographic sensitive body. The electrophotographic sensitive body was charged by a corona discharge at -7.0 kv. The decay of the surface potential in the dark was measured for each electrophotographic sensitive member (1) left in the dark place for sufficient time, (2) illuminated for 2 min. at 2000 lux with a fluorescent lamp and charged 15 sec. after the illumination finished, and (3) illuminated for 2 mins. at 2000 lux with a fluorescent lamp, and charged 5 min. after the illumination finished. Thus, consequently, the pre-exposure effect on decay in the dark is examined. Further, the photosensitivity is shown as a value of time which is required for half decay of the surface potential when the said body is illuminated at 15 lux of light intensity of 2660° K. tungsten lamp, after being charged at -7.0 kv. by a corona discharge.

When the content of photoconductive powder is decreased, the initial surface potential and decaying in the dark is improved, but the photosensitivity falls down. From the above relation, a content ratio of these compositions fit for an object could be determined. Still more, it would be understood from the table that a pre-exposure effect could hardly be recognized. Although in the above examples of this invention an aluminum plate is employed as a backing member, the said member should not be restricted to aluminum. Other material could be used as the substrates. Because of employing a binder material that

can be dried to form a hard layer at room temperature, a poor thermostable substrate such as paper or plastics may be used to produce a photosensitive member. Further, this paint can be coated over such a plate that can hardly be heated, for example, iron or steel plate, to form a large electrophotographic photosensitive plate.

Further, it is similar to other photosensitive insulating material comprising a photoconductive powder and a resin binder in which many other kinds of thermoplastic resins and thermosetting resins are widely usable. Further, a glass material could be employed.

In a series of photoconductive powders comprising various content ratios of cadmium sulfide and cadmium carbonate, the most preferred have the formula



wherein  $n$  has a value up to about 4, taking their characteristics into consideration. Materials whose content ratios lie beyond above range, are of course usable, though their properties fall behind. It is also possible to add some impurities to the said material of the composition. In particular, oxygen has been observed as a form of cadmium oxide in the powder of an example of this invention. Also, the existence of a trace of selenium, as cadmium selenide, is allowed.

What is claimed is:

1. A method for producing a photoconductive insulating material comprising firing a mixture of cadmium carbonate and sulfur to produce a material represented by the formula



where  $n$  is greater than 0 and has a value up to about 4, forming a dispersion of  $\text{CdS} \cdot n\text{CdCO}_3$  in a resinous binder and solvent for the binder, coating said dispersion on a substrate, and drying and thermally curing said coating.

2. A photoconductive insulating material comprising an electrically insulating binder material having a bulk resistivity of at least  $10^{11}$  ohms-cm. at room temperature, and finely divided particles of a photoconductive material dispersed in said binder material, said photoconductive material being represented by the formula



in which  $n$  represents  $0 < n \leq 4$ .

## References Cited

## UNITED STATES PATENTS

|           |         |             |           |
|-----------|---------|-------------|-----------|
| 2,959,481 | 11/1960 | Kucera      | 96—1      |
| 3,234,017 | 2/1966  | Heyl et al. | 117—201 X |
| 3,251,714 | 5/1966  | Rotschild   | 117—201   |

WILLIAM L. JARVIS, Primary Examiner

U.S. Cl. X.R.